

## UNITED STATES PATENT OFFICE

1,929,205

## PAPER MAKING

Clarence Earl Libby, Syracuse, N. Y., assignor to  
 National Aluminate Corporation, Chicago, Ill.,  
 a corporation of Delaware

No Drawing. Application April 4, 1932  
 Serial No. 603,223

13 Claims. (Cl. 92—21)

The present invention relates to an improved process for the manufacture of paper, cardboard, pulp-board and the like, having special reference to the sizing and web-forming steps.

- 5 One of the major objects of the invention is to improve the efficiency of the sizing operation, as well as to diminish the amounts of sizing-reagents required to bring a given type of paper to a predetermined degree of size resistance.
- 10 A further object of the invention is to treat cellulosic fibers that are suspended in water in a beater with a water-soluble aluminate for the purpose of neutralizing the water to a point where the size, when subsequently added, will be more 15 efficiently dispersed so that, when it is later precipitated upon the fiber by the addition of the usual precipitants, such as aluminum sulphate, a much more thorough sizing of the fibers will result. A secondary, but valuable, result is 20 obtained by the use of the aluminate in that the resulting sized stock is considerably freer, so that the speed of web production can be considerably increased, while there will also be less loss of fiber in the white-water.
- 25 Other objects will become apparent as the invention is further described.

The invention therefore may be summed up as consisting of the process of improving the sizing operation in paper manufacture by the adjustment of the acidity or hydrogen ion concentration of the water in the beater to about the point of neutrality (pH 7.0) by means of a soluble aluminate, followed by addition of the size and, later, by the usual aluminum sulphate. Ex- 35 act neutrality need not be attained, the useful range being between pH 5.0 to pH 8.0.

In this connection it should be understood that the action of the sodium aluminate is not one of mere neutralization, for, as will be shown in 40 detail hereinbelow, the effects obtained can not be interpreted merely upon the alkalinity of the sodium aluminate.

Paper is sized for the purpose of making it 45 resistant to the penetration of water, ink, oil, or other fluids. Ordinarily, sizing is accomplished by introducing into the paper sheet a water resistant material such as rosin, glue, casein, or paraffin wax. Rosin is the most common and efficient sizing material and is used in far greater 50 quantities for this purpose than all other materials combined.

Rosin itself is not soluble in water but is 55 brought into a soluble state by treatment with an alkali, the solution being accomplished either with or without the application of heat. The re-

sulting thick "rosin soap", so called, may be added directly to the paper pulp beaters but is more commonly "emulsified" or diluted with water to a concentration of 2% to 5% before it is added to the pulp stock. After the addition of the 60 rosin emulsion, the size is usually "set" or fixed on the fibers by the addition of aluminum sulphate, or paper makers' alum, although in special cases the alum is added before the rosin size.

Notwithstanding the apparent simplicity of this 65 operation, the practical results obtained are often quite variable and sometimes so unsatisfactory that the finished paper cannot be utilized for the intended purpose. It is possible to add the proper amount of size and alum in the correct manner 70 and produce no increase in the size resistance of the paper over the unsized pulp, i. e., the efficiency of the operation has been zero. While this result would seem unusual, it is not unusual, and in fact it is common for the size resistance 75 of a given sheet manufactured in a single mill to vary in size resistance from run to run, from day to day, and even, in some cases, from hour to hour as much as several hundred percent.

I have found that the greatest cause of this 80 fluctuation in size resistance is due to a varying acidity of the pulp suspension in the beater. The dispersion of the colloidal rosin size suspension is affected by this acid condition at the moment of addition to the beater, and the result- 85 ing size resistance of the paper manufactured from this pulp is a function of the dispersion of this size. Other factors being constant and within well defined limits, the greater the acidity of the pulp at the time of addition of the size, the 90 less will be the size resistance of the manufactured paper. The variation in acidity of the pulp beaters is due to a number of factors, chief among which may be mentioned residual acid from the liquors in which the wood was cooked, 95 acid from the bleaching operation, free acid from the alum and mineral filler which has accumulated in the white water, this water ordinarily being reused for dilution in the beaters, and acid resulting from the true hydrolysis of the alum- 100 in sulphate.

The process which I have developed for the use of sodium aluminate in connection with the sizing operation depends in part on the power of the aluminate to neutralize the pulp stock acidity 105 and thereby create more favorable conditions for the dispersion of the rosin size emulsion.

In practice the pulp suspension in the beater will have an acidity, expressed in terms of pH units, ranging from pH 3.5 to pH 8.5, depending 110

upon the combination of factors enumerated heretofore and upon whether the pulp stock was prepared by an acid or an alkaline process. If the pulp was prepared by an acid process, or has been subjected to a bleaching treatment, or is suspended in the white water which drains away from the paper machine wires, it will have, ordinarily, an acidity not greater than pH 6.0 and probably not greater than pH 5.0. It is my process to adjust this acidity to approximate neutrality (pH 7.0) by the addition of sodium aluminate, although in special cases the adjusted acidity varies from pH 5.0 to pH 8.0. The rosin size emulsion is then added and after thorough agitation the mixture of rosin and aluminate is precipitated throughout the pulp stock by the addition of sufficient aluminum sulphate or other acid salt to adjust the acidity back to pH 4.0 or whatever figure has been determined to give maximum sizing results.

The use of sodium aluminate for this purpose is original with me and gives results which cannot be obtained with any other alkaline salt, these results being due in part to the neutralizing power of the aluminate and in part to the colloidal floc resulting from the interaction of the aluminate and the residual acid or aluminum sulphate dissolved in the water of the pulp suspension. This floc being of itself a colloid serves to disperse the rosin size emulsion and greatly assists in the even distribution and uniform sizing of the entire paper sheet.

It is also evident that the presence of the aluminate causes a more complete precipitation of the rosin size, which brings about a greater retention of rosin size in the sheet and results in less loss of size and alum in the machine white waters. This enables a mill to greatly reduce the amount of rosin size addition to obtain a given degree of sizing or size resistance in their paper and results in significant economies in the manufacturing process. If a mill is unable to manufacture a satisfactorily sized paper without aluminate, the addition of this chemical will increase the degree of sizing in their product to a satisfactory value and thereby enable the mill to manufacture more salable merchandise.

In addition to the aforementioned benefits, the flocculating power of the aluminate added to the beater causes an agglomeration of the fine fibers in the pulp suspension, these fine fibers being trapped by the aluminate floc and the whole mass enmeshed in the fiber structure of the paper sheet in a manner which prevents these fine fibers from passing through the fiber mat of the wet paper sheet on the machine wire and subsequently through the machine wire itself, resulting in a marked decrease in the loss of fine fibers in the white water effluent going to the sewers.

Furthermore, the addition of sodium aluminate to any paper pulp stock gives in some cases a soft flexible paper sheet similar to a wood fiber prepared by the soda chemical pulping process and highly desirable for the manufacture of bookpapers. By closely regulating the initial and final conditions of acidity, together with the time of treatment in the beaters, exactly the opposite effect may be produced, at will, and a stiff strong paper sheet similar in characteristics to a rag paper sheet, may be manufactured from wood or other fibers of inferior initial strength and less economic value than the rag fibers which they simulate.

The addition of aluminate to the pulp stock in the beaters, or at any other point in the line

of flow of this pulp stock to the paper machine, develops a highly desirable characteristic in the pulp stock known as "freeness." The development of this freeness characteristic gives to the pulp stock several valuable properties greatly desired by the paper makers, for example:

(a) It dissipates the darker color of hydrated pulp stock and gives a decidedly lighter color to undyed pulp, resulting in a brighter and lighter color in the finished paper than would otherwise be the case.

(b) It permits the fibers to form or "felt" more quickly on the paper machine wire and results in a more dense, uniform, and finely knit sheet known to the paper makers as a sheet with "closed" formation.

(c) It enables the felts, suction boxes, and presses of the paper machine to remove with less difficulty the suspension water associated with the fibers and permits the paper machine to be operated at decidedly greater speeds.

(d) It enables the paper machine dryers to evaporate the residual water in the wet sheet leaving the presses with a smaller amount of steam, resulting in decreased drying costs and also permitting greater operating speeds, as the speed of the operation of a paper machine is often determined by its drying capacity.

(e) It largely negates the tendency of hydrated pulp stock to shrink as it dries on the rotating steam-heated drying drums of the paper machine and permits a machine to manufacture a sheet of greater width than would be possible without the use of sodium aluminate.

The results of tests made on an operating scale, using sodium aluminate in the beaters, with the object of increasing the efficiency of the sizing operation, will now be described.

These tests were made during a regular run of 16 point board, and, as a previous test had indicated that a substantial increase in the size test results from the addition of aluminate, an immediate cut of 25% in both the size and alum furnish was made simultaneously with the addition of aluminate. The size and alum furnish per beater during this test was as follows:

| Ply               | Size    | Alum    | Aluminate |
|-------------------|---------|---------|-----------|
| Top liner.....    | 40 lbs. | 50 lbs. | 4 lbs.    |
| Bottom liner..... | 45 lbs. | 55 lbs. | 4 lbs.    |

The effect of this aluminate addition on sizing efficiency can be judged from the following summary of the penetrometer size tests on boards manufactured under the conditions described.

1. Previous standard size test on 16 point board according to present physical standards—8 min. 30 sec.

2. Size test on board manufactured with a cut of 25% in both size and alum furnish but with 4 lbs. solid sodium aluminate in each liner beater—18 min. 18 sec.

3. Size test on board manufactured with a cut of 25% in both size and alum furnish, but with 4 lbs. of liquid sodium aluminate, (based on  $Al_2O_3$  content) in each liner beater—7 min. 54 sec.

An inspection of the foregoing tests indicates that a marked increase in sizing accompanies the use of solid sodium aluminate but that the liquid aluminate is not quite so effective, although the present standard test was practically maintained with this product even after a 25% cut in size and alum.

In order further to test the advantages resulting from the use of sodium aluminate in the beaters in connection with the manufacture of paper, three runs were made, one using ordinary 5 fresh lake water having an initial hydrogen-ion concentration of pH 6.4, and when treated with the alum used for the precipitation, of pH 4.2. The size test in this case was 106 seconds. A second run was then made with the use of the 10 white-water from the first run in the beaters, so that the water in the beater had an initial hydrogen-ion concentration of pH 4.2 both before and after addition of the necessary paper-marker's alum to effect the precipitation. The size test 15 in this case was only 80.1 seconds.

A third run was then made, employing the white-water from run No. 2, which had an initial hydrogen-ion concentration of pH 4.2. Sufficient 20 sodium aluminate was then added to bring the hydrogen-ion concentration of the water in the beater to the neutral point, i. e., pH 7.0. Thereupon the regular amount of size was added and the size precipitated by means of alum, in exactly the way it had been done with the two 25 preceding runs. The size test on the resulting paper was 277.4 seconds, or an increase over run No. 2 of 246%. It is thus plainly evident that the addition of the aluminate very greatly increased the size resistance of the paper.

In order to obtain still more convincing proof 30 of the remarkable effect obtained when practicing the present invention, a number of further test runs were made. These were as follows:

*Run No. 4.*—A run made for the purpose of 35 preparing white water and employing a furnish of fresh water, rosin size, sodium aluminate and alum.

*Run No. 5.*—A run made for the purpose of 40 preparing white water and employing a furnish of white water from Run No. 4, rosin size, sodium aluminate and alum.

*Run No. 6.*—A run made for the purpose of 45 determining the specific effect of sodium aluminate on the efficiency of the rosin sizing operation and employing a furnish of white water from Run No. 5, rosin size, sodium aluminate and alum.

In order to prove that the effect obtained 50 could not be ascribed merely to the neutralization of the white-water used in the beater, three further test runs were made, using sodium carbonate as the neutralizing medium. These were as follows:

*Run No. 7.*—A run made for the purpose of 55 preparing white water and employing a furnish of fresh water, rosin size, sodium carbonate and alum.

*Run No. 8.*—A run made for the purpose of 60 preparing white water and employing a furnish of white water from run No. 7, rosin size, sodium carbonate and alum.

*Run No. 9.*—A run made for the purpose of 65 determining the specific effect of sodium carbonate on the efficiency of the rosin sizing operation and employing a furnish of white water from Run No. 8, rosin size, sodium carbonate and alum.

The details of these runs are as follows:

#### Run No. 4

Pulp—100% Dexter bleached mitscherlich sulphite pulp.  
Pulp furnish—10 lbs. air dry at 5% consistency.  
Beating time—Two hours, fifteen minutes.  
Beater roll setting—38 on Bristol recorder.

Water—Fresh water having a pH of 6.4.  
Rosin size—Paper Makers Chemical Corp., 80% solids, 18% free rosin.  
Rosin size furnish—5% of 60% size or 3% on air dry weight of pulp.  
Aluminate—Dissolved C. P. sodium aluminate added after fifteen minutes of beating in sufficient quantity to increase the pH of the pulp suspension in the beater to a pH of 7.0 rosin size then added to the beater.  
Aluminate furnish—The equivalent of 4.4 lbs. of dry C. P. sodium aluminate per ton of air dry pulp.  
Alum—Dissolved C. P. aluminum sulphate added after one hour fifty-five minutes of beating in sufficient quantity to adjust the acidity of the pulp in the beater to a pH of 4.2.  
Alum furnish—The equivalent of 88.2 lbs. of C. P. aluminum sulphate per ton of air dry pulp.  
Green's freeness test—None.  
Test sheets—None.  
Valley size test—None.

#### Run No. 5

Pulp—100% Dexter bleached mitscherlich sulphite pulp.

Pulp furnish—10 lbs. air dry at 5% consistency.  
Beating time—Two hours, fifteen minutes.

Beater roll setting—38 on Bristol recorder.  
Water—White water from Run No. 4, having an initial pH of 4.2.

Rosin size—Paper Makers Chemical Corp., 60% solids, 18% free rosin.

Rosin size furnish—5% of 60% size, or 3% rosin on air dry weight of pulp.

Aluminate—Dissolved C. P. sodium aluminate added after fifteen minutes of beating and in sufficient quantity to increase the pH of the pulp suspension in the beater from pH 4.2 to a pH of 7.0. Rosin size then added to the beater.

Aluminate furnish—The equivalent of 18.7 lbs. of dry C. P. sodium aluminate per ton of air dry pulp.

Alum—Dissolved C. P. aluminum sulphate added after one hour fifty minutes of beating and in sufficient quantity to adjust the acidity of the pulp in the beater to a pH of 4.2.

Alum furnish—The equivalent of 88.2 lbs. of C. P. aluminum sulphate per ton of air dry pulp.

Green's freeness test—None.  
Test sheets—None.

Valley size test—None.

#### Run No. 6

Pulp—100% Dexter bleached mitscherlich sulphite pulp.

Pulp furnish—10 lbs. air dry at 5% consistency.  
Beating time—Two hours, fifteen minutes.

Beater roll setting—38 on Bristol recorder.  
Water—White water from Run No. 5, having an initial pH of 4.2.

Rosin size—Paper Makers Chemical Corp., 60% solids, 18% free rosin.

Rosin size furnish—5% of 60% size, or 3% rosin on the air dry weight of pulp.

Aluminate—Dissolved C. P. sodium aluminate added after fifteen minutes of beating in sufficient quantity to increase the pH of the pulp suspension in the beater to a pH of 7.0. Rosin size then added to the beater.

|     |                                                                                                                                                                                                                                   |     |
|-----|-----------------------------------------------------------------------------------------------------------------------------------------------------------------------------------------------------------------------------------|-----|
| 5   | Aluminate furnish—The equivalent of 18.7 lbs. of C. P. sodium aluminate per ton of air dry pulp.                                                                                                                                  |     |
| 10  | Alum—Dissolved C. P. aluminum sulphate added after one hour fifty-five minutes of beating in sufficient quantity to adjust the acidity of the pulp in the beater to a pH of 4.2.                                                  |     |
| 15  | Alum furnish—The equivalent of 88.2 lbs. of C. P. aluminum sulphate per ton of air dry pulp.                                                                                                                                      |     |
| 20  | Green's freeness test—None.                                                                                                                                                                                                       |     |
| 25  | Test sheets—Formed on Bureau of Standards sheet machine and air dried at 70° F.                                                                                                                                                   |     |
| 30  | Test sheet weights—29.1 grams for 4 sheets 8" x 10".                                                                                                                                                                              |     |
| 35  | Valley size test data obtained at 70° F. and 65% relative humidity.                                                                                                                                                               |     |
| 40  | Seconds                                                                                                                                                                                                                           |     |
| 45  | Sample 1-----180                                                                                                                                                                                                                  |     |
| 50  | Sample 2-----182                                                                                                                                                                                                                  |     |
| 55  | Sample 3-----191                                                                                                                                                                                                                  |     |
| 60  | Sample 4-----148                                                                                                                                                                                                                  |     |
| 65  | Sample 5-----190                                                                                                                                                                                                                  |     |
| 70  | Sample 6-----162                                                                                                                                                                                                                  |     |
| 75  | Sample 7-----196                                                                                                                                                                                                                  |     |
| 80  | Sample 8-----205                                                                                                                                                                                                                  |     |
| 85  | Sample 9-----145                                                                                                                                                                                                                  |     |
| 90  | Sample 10-----165                                                                                                                                                                                                                 |     |
| 95  | Average-----176.4                                                                                                                                                                                                                 |     |
| 100 | Run No. 7                                                                                                                                                                                                                         |     |
| 105 | Pulp—100% Dexter bleached mitscherlich sulphite pulp.                                                                                                                                                                             |     |
| 110 | Pulp furnish—10 lbs. air dry at 5% consistency.                                                                                                                                                                                   |     |
| 115 | Beating time—Two hours, fifteen minutes.                                                                                                                                                                                          |     |
| 120 | Beater roll setting—38 on Bristol recorder.                                                                                                                                                                                       |     |
| 125 | Water—Fresh water having a pH of 6.4.                                                                                                                                                                                             |     |
| 130 | Rosin size—Paper Makers Chemical Corp., 60% solids, 18% free rosin.                                                                                                                                                               |     |
| 135 | Rosin size furnish—5% of 60% size, or 3% rosin on the air dry weight of pulp.                                                                                                                                                     |     |
| 140 | Aluminate—None.                                                                                                                                                                                                                   |     |
| 145 | Soda ash—Dissolved C. P. sodium carbonate added after fifteen minutes of beating and in sufficient quantity to increase the pH of the pulp suspension in the beater from 6.4 to a pH of 7.0. Rosin size then added to the beater. |     |
| 150 | Soda ash furnish—The equivalent of 8.9 lbs. of C. P. sodium carbonate per ton of air dry pulp.                                                                                                                                    |     |
| 155 | Alum—Dissolved C. P. aluminum sulphate added after one hour fifty-five minutes of beating and in sufficient quantity to adjust the acidity of the pulp in the beater to a pH of 4.2.                                              |     |
| 160 | Alum furnish—The equivalent of 88.2 lbs. of C. P. aluminum sulphate per ton of air dry pulp.                                                                                                                                      |     |
| 165 | Green's freeness test—None.                                                                                                                                                                                                       |     |
| 170 | Test sheets—Formed on Bureau of Standards sheet machine and air dried at 70° F.                                                                                                                                                   |     |
| 175 | Test sheet weights—30.5 grams for 4 sheets 8" x 10".                                                                                                                                                                              |     |
| 180 | Valley size test data obtained at 70° F. and 65% relative humidity.                                                                                                                                                               |     |
| 185 | Seconds                                                                                                                                                                                                                           |     |
| 190 | Sample 1-----125                                                                                                                                                                                                                  | 135 |
| 195 | Sample 2-----135                                                                                                                                                                                                                  |     |
| 200 | Sample 3-----120                                                                                                                                                                                                                  |     |
| 205 | Sample 4-----107                                                                                                                                                                                                                  |     |
| 210 | Sample 5-----118                                                                                                                                                                                                                  |     |
| 215 | Sample 6-----122                                                                                                                                                                                                                  | 140 |
| 220 | Sample 7-----115                                                                                                                                                                                                                  |     |
| 225 | Sample 8-----134                                                                                                                                                                                                                  |     |
| 230 | Sample 9-----110                                                                                                                                                                                                                  |     |
| 235 | Sample 10-----105                                                                                                                                                                                                                 | 145 |
| 240 | Average-----119.1                                                                                                                                                                                                                 |     |
| 245 | The procedures followed in making the runs just described were identical with those employed in making runs Nos. 1-3. However, it was decided to make an accurate check on the quantity of                                        | 150 |

aluminate, soda ash, and alum used as well as on the pH obtained, and the data obtained from these measurements are tabulated and discussed in the description to follow.

- 5 Owing to the considerable length of time required to complete these six runs, it was decided to omit the freeness test, as this test is quite time consuming and as very little variation in freeness could be expected when such close control was 10 maintained over the beater roll setting and the time allowed for hydration.

It will be quite obvious to those skilled in this art that the precise sequence of the addition of the materials need not be followed. For example, 15 it would be an equivalent to add the aluminate to the water before mixing the fibers therewith; or to add the aluminate to the water, followed by addition of the size, and then to introduce the fibers. A third alternative is to add the fiber and 20 aluminate and size simultaneously. In any event, the complete or partial neutralization of the water by the aluminate will aid in the proper dispersion of the size and in the beneficial results obtained by the use of the present invention.

25 A summary of all of the test results obtained is herewith tabulated, so as to bring out most clearly the advantages of the present invention:

*Effect of the use of sodium aluminate and of sodium carbonate on paper sizing*

| Run No. | Beater water furnish |        | Neutralizing agent in # | Beater water pH |         | Size precip. in lbs. | Size test in sec. | % increase over run 2 | 105 |
|---------|----------------------|--------|-------------------------|-----------------|---------|----------------------|-------------------|-----------------------|-----|
|         | Nature               | Source |                         | Init.           | Tr'ted. |                      |                   |                       |     |
| 35      | 1 Fresh              | Lake   | None                    | 6.4             | 4.2     | Alum                 | 106               | 33%                   | 110 |
|         | 2 White              | Run 1  | None                    | 4.2             | 4.2     | Alum                 | 80.1              |                       |     |
|         | 3 White              | Run 2  | Aluminate q. s.         | 4.2             | 7.0     | Alum                 | 277.4             | 246%                  |     |
|         | 4 Fresh              | Lake   | Aluminate 4.4           | 6.4             | 7.0     | Alum 88.2            | Not run           |                       |     |
|         | 5 White              | Run 4  | Aluminate 18.7          | 4.2             | 7.0     | Alum 88.2            | Not run           |                       |     |
|         | 6 White              | Run 5  | Aluminate 18.7          | 4.2             | 7.0     | Alum 88.2            | 176.4             | 120%                  |     |
|         | 7 Fresh              | Lake   | Soda ash 2.2            | 6.4             | 7.0     | Alum 88.2            | Not run           |                       |     |
|         | 8 White              | Run 7  | Soda ash 8.9            | 4.2             | 7.0     | Alum 88.2            | Not run           |                       |     |
|         | 9 White              | Run 8  | Soda ash 8.9            | 4.2             | 7.0     | Alum 88.2            | 119.1             | 49%                   |     |

The foregoing test data explains the reason why the test values obtained for Run No. 3 in the first series of runs were abnormally high due to the fact that the white water for this run had not had previous treatment with aluminate. As will be noted, the test values for Run No. 6, which is identical with Run No. 3 except that the white water for Run No. 6 had been treated twice previously with sodium aluminate, shows an increase in sizing value of 120% over Run No. 2, the run in which the pulp stock was sized while suspended in unneutralized white water. This test value of 120% corresponds with the test value of 246% obtained for Run No. 3, the run in which the white water had not been treated previously with aluminate. These comparative results furnish positive evidence that the function of the aluminate in increasing sizing efficiency is due to its ability to bring about a more complete precipitation and retention of the rosin size in the paper sheet, thereby clearing the white water of dissolved size and alum, and making possible a decided reduction in size furnish to obtain a given size test value.

The effect of soda ash in increasing sizing efficiency is shown by the size test value obtained from Run No. 9. These test values indicate a degree of sizing 49% greater than the values from Run No. 2. These figures indicate further that sodium aluminate has approximately three times the beneficial effect of soda ash in increasing sizing efficiency.

The conclusions to be deduced from the foregoing tests are:

(a) That the neutralization of beater acidity with sodium aluminate prior to the addition of rosin size has a marked beneficial effect on sizing efficiency.

(b) That the beneficial effect of sodium aluminate is partially if not wholly due to a more complete precipitation and retention of the rosin size in the paper sheet and a resulting cleaner white water.

(c) That the neutralization of beater acidity with sodium carbonate prior to the addition of rosin size has an effect somewhat similar to that of sodium aluminate, but that the efficiency of sodium carbonate as a neutralizing agent is apparently only one-third that of sodium aluminate.

It will thus be seen that the size resistance of paper can be increased from 120 to 277.4% by the use of sodium aluminate for neutralizing the white water when the same is used in making up the furnish for the beaters. When, on the contrary, sodium carbonate is used for a somewhat similar purpose, namely, to bring the white water to the neutral point before adding the size, and then precipitating the size by means of the usual papermakers alum (aluminate sulphate), the increase in size-resistance is only 49%. It

will thus be quite apparent that a considerable step has been made in advancing this particular part of the art of paper making.

Reserving unto himself the benefits of the use of such equivalents as will occur to the experienced chemist and papermaker, what applicant has invented and claims is as follows:

1. The process of sizing cellulosic fibers for the production of webs therefrom, which comprises treating the fibers in suspension with size and a water-soluble alkaline aluminate, and thereupon precipitating the size upon the fibers by means of an acid-reacting soluble reagent.

2. The process of sizing cellulosic fibers for the production of webs therefrom, which comprises treating the fibers in aqueous suspension with sodium aluminate and a size, and thereupon precipitating said size upon the fibers by the addition of an alum.

3. The process of sizing cellulosic fibers for the production of webs therefrom, which comprises treating the fibers in aqueous suspension with sodium aluminate and a size, and thereupon precipitating said size upon the fibers by the addition of aluminum sulphate.

4. The process of sizing cellulosic fibers which comprises treating the same first with a mixture of a rosin size and sodium aluminate, and thereupon precipitating both the sodium aluminate and the size by the addition of aluminum sulphate.

5. The process of sizing cellulosic fibers which comprises treating the same with a solution of a rosin size and sodium aluminate, and then acidifying.

- fyng the solution by means of an acid-reacting salt.
6. The process of increasing the size-resistance of paper which consists in suspending cellulosic fibers in water that has been neutralized by the addition of sodium aluminate, adding a rosin size to the suspension, and thereupon acidifying the suspension by the addition thereto of an acid-reacting salt.
- 10 7. The process of increasing the size resistance of paper, which consists in suspending cellulosic fibers and size in water that has been neutralized with sodium aluminate, and thereupon acidifying the resultant suspension by the addition of aluminum sulphate.
- 15 8. In the process of manufacturing paper from cellulosic fibers which are suspended in the white-water from a previous run of paper-manufacture, the step of neutralizing said white-water by the addition thereto of sufficient sodium aluminate to bring the suspension to substantially the neutral point, adding size to the suspension, and precipitating said size upon the fibers.
- 20 9. The process of neutralizing white-water which comprises adding sufficient sodium aluminate thereto to bring it substantially to the neutral point.
- 25 10. In the manufacture of cellulosic webs the
- improvement which comprises suspending fibers in white-water, neutralizing the suspension with sodium aluminate, adding rosin size to the suspension, adding aluminum sulphate to the suspension, and thereupon sheeting the fibers into a coherent web.
11. In the manufacture of webs from fibers, the improvement which consists in suspending fibers in an aqueous medium that has a hydrogen-ion concentration above the neutral point, bringing said medium to substantial neutrality by the addition of sodium aluminate, adding a precipitable size to the resulting suspension, and then precipitating said size upon the fibers by means of an acid-reacting salt such as aluminum sulphate.
- 15 12. The process of enhancing the efficacy of rosin sizing of fibers, which comprises neutralizing the water in which the fibers are dispersed by means of sodium aluminate, adding dissolved rosin size, and thereupon adding aluminum sulphate to form an insoluble precipitate of size and aluminum compounds upon the fibers.
- 90 13. The process of manufacturing sized paper which comprises preparing a mixture of fibers, a soluble aluminate and a sizing-agent, and treating this mixture with an acid-reacting size-precipitating agent.
- 95 CLARENCE EARL LIBBY.
- 100
- 105
- 110
- 115
- 120
- 125
- 130
- 135
- 140
- 145
- 150
- 30
- 35
- 40
- 45
- 50
- 55
- 60
- 65
- 70
- 75